

Feb. 27, 1934.

E. GRAF

1,949,372

MAKING LEAD ALLOY CASTINGS

Filed Feb. 29, 1932



FIG. 1.



FIG. 2.



FIG. 3.

WITNESS:

Peter R. Kitchell.

INVENTOR  
*Ernest Graf*

BY

*Augustus B. Swegerton.*  
ATTORNEY.

## UNITED STATES PATENT OFFICE

1,949,372

## MAKING LEAD ALLOY CASTINGS

Ernest Graf, Philadelphia, Pa., assignor to The  
Electric Storage Battery Company, Philadel-  
phia, Pa., a corporation of New Jersey

Application February 29, 1932. Serial No. 595,966

## 1 Claim. (Cl. 22—136)

Lead alloy grids and plates for storage batteries are examples of intricate castings usually made in ferrous metal molds, containing intersecting mold cavities, and in making such castings it frequently happens that the molten lead alloy does not flow in such a way as to fill the mold, so that defective castings are produced. Attempts have been made to prolong the flow and to improve the castings by lubricating the polished metal faces of the mold and by heating the molds.

One object of the present invention is to overcome these defects and disadvantages and to provide for the production of perfect castings without the use of lubricants on the surfaces of the mold and without the application of heat to the molds, or with the application of less heat than heretofore. Another object is to give to the castings a fine grained and tough structure.

Generally stated, the invention consists in perceptibly roughening the metal surfaces of the intersecting channels of the mold and pouring the molten lead alloy in contact with such roughened metal surfaces.

The invention also comprises the improvements to be presently described and finally claimed.

In the practice of the invention the surfaces of the mold channels, which frequently intersect, if polished are depolished, or are otherwise made perceptibly rough, and the perceptible roughness of the metal mold surfaces in direct contact with the molten alloy cause the latter to flow further than it would do if in contact with polished metal mold surfaces, or with mold surfaces lubricated by the application of any lubricant with which I am familiar. Thus the intersecting channels of the mold space or the mold space itself is well filled and good castings, however intricate or elongated, are produced. In some cases the length of flow in a metal mold can be increased by heating the mold, and this is true in the case

of this invention, but in it less heat need be applied.

The metal surface of the mold may be perceptibly roughened or depolished by scarifying it.

The present invention permits of the use of a relatively cold mold, while at the same time the mold is properly filled and a cold mold produces a quick chilled casting which gives a fine grained and tough structure to the alloy.

The present invention reduces the cost of molding operations by eliminating the frequent application or renewal of the usual lubricant.

In the accompanying drawing

Figure 1 is a face view illustrating parts of one-half of a well known mold for storage battery grids and diagrammatically showing the invention.

Fig. 2 is a like view, and

Fig. 3 is an enlarged section on the line 3—3 of Fig. 1.

In the drawing the stipple indicates the perceptibly roughened metallic surfaces of the intersecting channels or cavities 1, Fig. 1, and of the cavities 2, Fig. 2.

It will be obvious to those skilled in the art to which the invention relates that modifications may be made in details of construction and mode of procedure without departing from the spirit of the invention which is not limited to such matters or otherwise than the prior art and the appended claim may require.

I claim:

For making intricate lead alloy castings, an operatively stationary mold of ferrous metal having internal intersecting channels provided with metal faces presenting perceptibly roughened metal surfaces for contact with the pour and which promote the progressive flow of molten alloy from channel to channel throughout the mold to completely fill the same.

ERNEST GRAF.